

## UNITED STATES PATENT OFFICE

2,437,063

## NONDIFFUSING 1-PHENYL-5-PYRAZOLONE COUPLERS FOR COLOR PHOTOGRAPHY

Walter Zeh, Wolfen, Kreis Bitterfeld, and Wilhelm Schneider and Alfred Fröhlich, Dessau, Germany, assignors to General Aniline & Film Corporation, New York, N. Y., a corporation of Delaware

No Drawing. Application February 17, 1942, Serial No. 431,263. In Germany August 8, 1940

7 Claims. (Cl. 95—6)

1

Our present invention relates to the production of color photographic images and more particularly to an improved photographic silver halide emulsion containing a dyestuff former.

In the production of color photographic images by color forming development it is already known to use dyestuff formers containing radicals producing fastness to diffusion and groups making the compounds soluble in water. For the production of red color tones it has, for instance, been proposed to use 1-phenyl-5-pyrazolones having radicals preventing diffusion and sulfo or carboxyl groups. Such pyrazolone is, for instance, 1-(phenyl-3'-sulfonic acid)-3-heptadecyl-5-pyrazolone which would be especially suitable for high-sensitive multi-layer materials owing to its high sensitivity if it did not show certain disadvantages. The high color yield of this dyestuff former is attended with a strong tendency to "bronze" the color tone and a certain tendency to produce color fogging. Furthermore, this dyestuff component yields images having a too steep gradation on color development. Therefore incorrectness in color reproduction is obtained when the component is employed in a multi-layer material.

It is an object of our present invention to obviate the above-mentioned drawbacks. Further objects will be apparent from the detailed specification following hereinafter.

These objects are accomplished by using a 1-phenyl-5-pyrazolone carrying a radical producing fastness to diffusion in the 3-position of the pyrazolone nucleus and one or several substituents in the 3-, 4- or 5-positions of the phenyl radical besides groups increasing the solubility in water. Useful substituents are alkyl, alkoxy, alkthio, alksereno, aryloxy, and halogens. The pyrazolones are prepared by reacting phenylhydrazine-sulfonic acids or phenylhydrazine carboxylic acids correspondingly substituted with high-molecular weight acylacetic acid esters. The pyrazolones substituted according to the invention are distinguished from the corresponding non-substituted pyrazolones by a slight tendency to produce color fogging and by the formation of non-bronzing dyestuffs the color tone of which is only inessentially displaced, on development with color forming developers without the high sensitivity being decreased. The red component images thus obtained show a less steep gradation than the color images from the corresponding non-sub-

2

stituted compounds so that the resulting multi-color images exhibit a red tint well graduated.

The phenylpyrazolones of the present invention contain in the 3-position of the pyrazolone nucleus radicals preventing diffusion, for instance, carbon chains with at least 6 carbon atoms (see U. S. P. 2,186,849, dated January 9, 1940) or other radicals, for instance, those described in "Stenger-Staude, Fortschritte der Photographie, volume II, 1940, pages 393-397." Besides these substituents groups rendering the components soluble in water may also be present in the phenyl nucleus such as sulfo, carboxyl or hydroxyl groups.

The silver halide emulsion prepared by means of the dyestuff components of the present invention may be cast to form single layers or worked up into a multi-layer material containing further emulsion layers with dyestuff formers for the other component colors and, if necessary, filter layers, intermediate layers and anti-halation layers. The emulsion layers may contain corresponding sensitizers and be arranged on one or both sides of the support. The multi-layer material may also comprise emulsion layers capable of producing dyestuffs according to a color photographic method rather than that mentioned above. The color images may be obtained by a simple development or a reversal development as negatives or positives respectively.

The following examples illustrate the present invention but they are not intended to limit it thereto.

*Example 1*

35 10 g. of 1-(4'-methylphenyl-3'-sulfonic acid)-3-heptadecyl-5-pyrazolone are neutralized with a diluted sodium hydroxide solution with warming. The resulting solution of the sodium salt is made up to 200 cc. with water, then added to 1 kilo of a silver halide gelatin emulsion and finally cast. After exposure a non-bronzing slightly bluish-red dyestuff image having an absorption maximum at about 530 m $\mu$  is produced by treating with a developer of the following composition:

|    |                                |       |       |
|----|--------------------------------|-------|-------|
| 45 | Potassium carbonate            | grams | 75    |
|    | p-Dimethylaminoaniline sulfate | do    | 2.5   |
|    | Potassium bromide              | do    | 2.5   |
|    | Sodium sulfite                 | do    | 2.5   |
| 50 | Water                          | cc.   | 1,000 |

and subsequently removing the formed silver.

## Example 2

10 g. of the sodium salt of 1-(4'-bromophenyl-3'-sulfonic acid)-3-heptadecyl-5-pyrazolone are dissolved in 200 cc. of water with gentle heating and added to 1 kilo of a silver halide gelatin emulsion layer before casting. On color forming development with a developer containing p-dimethylaminoaniline one obtains a non-bronzing, clear and slightly bluish red dyestuff image. This dyestuff shows a maximum absorption of about 530 m $\mu$ .

## Example 3

10 g. of 1-(3'-chlorophenyl-4'-sulfonic acid)-3-heptadecyl-5-pyrazolone are neutralized with a diluted sodium hydroxide solution and dissolved while gently heating. The solution made up to 200 cc. with water is added to 1 kilo of a silver halide gelatin emulsion before casting. A slightly blue-red, clear dyestuff image having a maximum absorption at about 530 m $\mu$  is produced with a color forming developer containing p-dimethylaminoaniline.

## Example 4

10 g. of the sodium salt of 1-(4'-chlorophenyl-3'-carboxylic acid)-3-heptadecyl-5-pyrazolone are dissolved in 200 cc. of water with warming and added to 1 kilo of a silver halide emulsion before casting. The color forming development with a developer containing p-dimethylaminoaniline yields a red dyestuff image having a maximum absorption at about 540 m $\mu$ .

## Example 5

10 g. of 1-(4'-methoxyphenyl-3'-sulfonic acid)-3-heptadecyl-5-pyrazolone are neutralized with a diluted sodium hydroxide solution and dissolved while gently heating. The solution made up to 200 cc. with water is added to a molten silver halide gelatin emulsion whereupon the emulsion is cast to form a layer. The color forming development yields a non-bronzing blue-red image the dyestuff of which has an absorption maximum of about 528 m $\mu$ .

## Example 6

10 g. of 1-(4'-meththiophenyl-3'-sulfonic acid)-3-heptadecyl-5-pyrazolone are added to 1 kilo of a silver halide gelatin emulsion and cast according to Example 5. One obtains a blue-red image the dyestuff of which shows an absorption maximum of about 530 m $\mu$  on color forming development with p-dimethylaminoaniline.

## Example 7

10 g. of 1-(4'-phenoxyphenyl-3'-sulfonic acid)-3-heptadecyl-5-pyrazolone are neutralized with 30 cc. of a n/10 sodium hydroxide solution, dissolved with gentle heating, made up to 200 cc. and added to one kilo of a molten silver halide gelatin emulsion before casting. The exposed emulsion layer yields a blue-red dyestuff image having an absorption maximum of about 530 m $\mu$  on color forming development with a developer containing dimethylaminoaniline.

## Example 8

If instead of the dyestuff former mentioned in Example 7 1-(4'-phenoxyphenyl-3'-sulfonic acid)-3-heptadecyl-5-pyrazolone is used, a blue-red dyestuff image having a maximum absorption of 530 m $\mu$  is produced.

## Example 9

10 g. of 1-(3'-chloro-4'-methylphenyl-5'-sulfonic acid)-3-heptadecyl-5-pyrazolone is neutralized with a diluted sodium hydroxide solution. The clear solution obtained by heating is made up to 200 cc. with water, added to 1 kilo of a molten silver halide gelatin emulsion and cast. A blue-red very transparent dyestuff image having an absorption maximum of about 535 m $\mu$  is obtained by the treatment with a developer containing dimethylaminoaniline.

Instead of the sodium salts of the pyrazolones of the invention other soluble salts may also be used, especially alkali metal salts.

We claim:

1. A silver halide emulsion for color forming development containing as the dyestuff former for red a soluble salt of 1-phenyl-5-pyrazolone containing in the 3-position of the pyrazolone nucleus a radical producing fastness to diffusion and in the phenyl nucleus at least one group increasing the solubility in water and in the positions of said phenyl nucleus selected from the group consisting of the 3-, 4- and 5-positions at least one substituent selected from the class consisting of alkyl, alkoxy, alkthio, alksereno, aryloxy and halogens.

2. A silver halide emulsion for color forming development containing as the dyestuff former for red a soluble salt of 1-phenyl-5-pyrazolone containing in the 3-position of the pyrazolone nucleus a carbon chain having at least 6 carbon atoms and in the phenyl nucleus at least one group increasing the solubility in water and in the positions of said phenyl nucleus selected from the group consisting of the 3-, 4- and 5-positions at least one substituent selected from the class consisting of alkyl, alkoxy, alkthio, alksereno, aryloxy and halogens.

3. A silver halide emulsion for color forming development containing as the dyestuff former for red a water-soluble salt of 1-(4'-methylphenyl-3'-sulfonic acid)-3-heptadecyl-5-pyrazolone.

4. A silver halide emulsion for color forming development containing as the dyestuff former for red a soluble salt of 1-(4'-bromophenyl-3'-sulfonic acid)-3-heptadecyl-5-pyrazolone.

5. A silver halide emulsion for color forming development containing as the dyestuff former for red a soluble salt of 1-(4'-chlorophenyl-3'-carboxylic acid)-3-heptadecyl-5-pyrazolone.

6. A silver halide emulsion for color forming development containing as the dyestuff former for red a soluble salt of a 1-phenyl-5-pyrazolone containing in the 3-position of the pyrazolone nucleus a radical imparting fastness to diffusion in the binding agent of the silver halide emulsion and containing in the phenyl nucleus a group increasing the solubility of the compound in water and in only one of the positions of said phenyl nucleus selected from the group consisting of the 3-, 4- and 5-positions a substituent selected from the class consisting of alkyl, alkoxy, alkthio, alksereno, aryloxy and halogen.

7. A silver halide emulsion as defined in claim 2 wherein the substituent in the 3-position of said pyrazolone is an aliphatic carbon chain of at least 6 carbon atoms and said substituent is directly linked to the carbon atom of the pyrazolone in said 3-position.

WALTER ZEH.

WILHELM SCHNEIDER.

ALFRED FRÖHLICH.

5

## REFERENCES CITED

The following references are of record in the file of this patent:

## UNITED STATES PATENTS

| Number    | Name            | Date         |
|-----------|-----------------|--------------|
| 2,179,239 | Wilmanns et al. | Nov. 7, 1939 |

5

| Number    |
|-----------|
| 2,186,849 |
| 2,200,306 |
| 2,213,986 |

6

| Name             | Date           |
|------------------|----------------|
| Wilmanns et al.  | Jan. 9, 1940   |
| Schneider et al. | May 14, 1940   |
| Kendall et al.   | Sept. 10, 1940 |

## FOREIGN PATENTS

| Number  | Country | Date          |
|---------|---------|---------------|
| 836,144 | France  | Oct. 10, 1938 |